



US005527600A

**United States Patent** [19]**Frankosky et al.**[11] **Patent Number:** **5,527,600**[45] **Date of Patent:** **Jun. 18, 1996**

[54] **BONDED POLYESTER FIBERFILL  
BATTINGS WITH A SEALED OUTER  
SURFACE**

2,454,391 11/1948 Jones et al. .... 427/366  
3,963,820 6/1976 Blakey .... 264/134  
4,551,383 11/1985 Sinischalchi .... 428/286  
4,869,771 9/1989 LeVan .... 156/289

[75] Inventors: **Michael S. Frankosky; Wo K. Kwok,**  
both of Hockessin, Del.

**FOREIGN PATENT DOCUMENTS**

[73] Assignee: **E. I. Du Pont de Nemours and  
Company**, Wilmington, Del.

A0265221A1 10/1987 European Pat. Off. .... D04H 1/42  
A0314433 10/1988 European Pat. Off. .... D04H 1/42  
A0437268A1 1/1991 European Pat. Off. .... D04H 1/64  
WO80/01031 2/1980 WIPO .  
WO93/11292 11/1992 WIPO .... D04H 1/64

[21] Appl. No.: **396,291**

*Primary Examiner*—Christopher W. Raimund

[22] Filed: **Feb. 28, 1995**

**ABSTRACT**

[63] Continuation-in-part of Ser. No. 84,936, Jul. 1, 1993, abandoned, which is a continuation-in-part of Ser. No. 800,177, Nov. 27, 1991, Pat. No. 5,225,242.

Improved polyester fiberfill batts for apparel and other uses are prepared of polyester fiber and binder fiber, sprayed with a soft resin by oven bonding and hot roll treatment. This provides bonded batting which is characterized by softness and drapability, good insulating performance, low levels of fiber leakage or percolation through shell fabrics, enhanced durability when laundered by washing/drying or by dry cleaning, and enhanced structural integrity whereby it hangs freely without the need for quilting into small size panels.

[51] **Int. Cl.<sup>6</sup>** .... **B32B 27/00**

[52] **U.S. Cl.** .... **428/286; 428/290**

[58] **Field of Search** .... 428/286, 290

[56] **References Cited**

**8 Claims, No Drawings**

**U.S. PATENT DOCUMENTS**

2,326,605 8/1943 Bass et al. .... 427/366

**BONDED POLYESTER FIBERFILL  
BATTINGS WITH A SEALED OUTER  
SURFACE**

**CROSS-REFERENCE TO RELATED  
APPLICATION**

This application is a continuation-in-part of application Ser. No. 08/084,936, which is being abandoned in favor of the present application, and which was filed Jul. 1, 1993, as a continuation-in-part of application Ser. No. 07/800,177 filed by Frankosky et al Nov. 27, 1991, and now issued as U.S. Pat. No. 5,225,242 on Jul. 6, 1993.

**FIELD OF THE INVENTION**

This invention is concerned with improvements in and relating to bonded polyester fiberfill batts, sometimes referred to as battings, especially processes whereby such improved batts with desirable aesthetic and serviceable qualities may be obtained, and to articles incorporating such improved batts.

**BACKGROUND OF THE INVENTION**

Polyester fiberfill (sometimes referred to as polyester fiberfilling material) is well accepted as a reasonably inexpensive filling and/or insulating material for pillows, cushions and other furnishing materials, including bedding materials, and in apparel, and is manufactured and used in large quantities commercially. For many of these uses, as disclosed, e.g., in U.S. Patents: Tolliver U.S. Pat. No. 3,772,137; Stanstreet U.S. Pat. No. 4,068,036; Scott U.S. Pat. No. 4,129,675; Pamm U.S. Pat. No. 4,281,042; Frankosky U.S. Pat. No. 4,304,817; Siniscalchi U.S. Pat. No. 4,551,383; and LeVan U.S. Pat. No. 4,869,771, it has been desirable to make bonded batts, e.g., by spraying a resin-bonding agent, usually of an acrylic polymer, or by blending the polyester fiberfill with binder fibers, such as are well known in the art, or by use of both a resin-bonding agent and binder fibers.

To improve the aesthetics of polyester fiberfill, it has often proved desirable to "slicken" the fiberfill with a coating of durable (i.e., wash-resistant) coating that has usually been a silicone, i.e., a cured polysiloxane as disclosed, e.g., by Hofmann U.S. Pat. No. 3,271,189; Mead et al U.S. Pat. No. 3,454,422; Ryan U.S. Pat. No. 3,488,217; Salamon et al U. S. Pat. 4,146,674; LeVan, above; Takemoto Oil and Fat Co., Ltd., Japanese Published Application No. 58-214, 585(1983); or other types such as the polyalkylene oxide variety disclosed by, e.g., Marcus U.S. Pat. No. 4,818,599.

Despite all the prior suggestions and commercially-available materials, especially for use in premium level apparel products, sleeping bags, and comforters, there still remains a need for an easily prepared, homogeneous batting that is characterized by softness and drapability to conform to the wearer's body, good insulating performance, low levels of fiber leakage through shell fabrics, even after laundering, enhanced durability to laundering by washing/drying or by dry cleaning, and enhanced structural integrity whereby the batting is able to hang freely without the need for having it quilted into small size panels.

**SUMMARY OF THE INVENTION**

According to one aspect of the invention, there is provided a process for preparing a bonded batt, comprising forming a blend of polyester fiberfill, in amount by weight about 70 to about 96%, intimately mixed with a binder fiber,

preferably a bicomponent binder fiber, having binder material of melting point lower than the softening point of the polyester fiberfill, in amount by weight about 4 to about 30%, preparing a continuous batt from said blend, said batt having an upper face and a lower face, advancing said batt through one or more spray zones, whereby both faces of the batt are sprayed with resin, in total amount about 10 to about 30% of the weight of the sprayed batt, including the resin, said resin being selected to provide, after curing, a cured resin having a glass transition temperature (Tg) of about 0 degrees Celsius or less, heating the sprayed batt in an oven to cure the resin and soften the binder material, followed by hot-rolling the heated batt to achieve intimate contact between the resin and the fibers in the faces of the batt, and cooling the rolled batt.

Such hot-rolling for this aspect of the invention is preferably effected by use of heated rolls in a calender or S-wrap configuration. The weight of the fibers in the batt (i.e., of the blend of polyester fiberfill and of binder fiber) is referred to as the "basis weight" of the batt, i.e., before the sealing resin is sprayed on.

Another aspect of the invention accordingly provides a bonded batt, comprising primarily polyester fiberfill of 0.2 to 10 dtex per filament (in amount about 75 to about 98%), bonded throughout with lower melting binder material (from the binder fiber used in the process) in complementary amount by weight about 2 to about 25% of the weight of the batt, and with upper and lower faces of said batt being sealed with a resin having a glass transition temperature (Tg) of about 0 degrees Celsius or less, and preferably from about 0 degrees down to about -30 degrees Celsius, in amount about 10 to about 30% of the weight of the batt, whereby the sealing rating (SR, as defined) of said faces is at least 3, said batt having a wash durability (WD, as defined) of at least 3, and a bending stiffness (B, as defined) of about 80 cN/cm<sup>2</sup> or less, preferably about 50 cN/cm<sup>2</sup> or less.

In addition to such bonded batts, that are sealed with resin on both faces, such as are generally preferred, there are also provided, according to another aspect, similar batts that are sealed on only one face, and containing half such amount of resin. Accordingly, there is provided a bonded batt with upper and lower faces, said batt comprising polyester fiberfill of 0.2 to 10 dtex per filament, in amount about 75 to about 98%, and bonded throughout with lower melting binder material, complementally in amount about 2 to about 25%, said amounts being calculated on the basis weight of the batt, said batt having a wash durability (WD, as defined) of at least 3, and a bending stiffness (B, as defined) of about 80 cN/cm<sup>2</sup> or less, wherein at least one of said faces is sealed with a resin having a glass transition temperature (Tg) of about 0 degrees Celsius or less, and preferably from about 0 degrees down to about -30 degrees Celsius, in amount about 5 to about 15% of the total weight of the batt, whereby the sealing rating (SR, as defined) of said face is at least 3.

According to a further aspect, hot rolling need not necessarily be performed to impart adequate sealing, by using low denier fiberfill (referred to variously as subdenier or microfibers) at least in one or both face(s) of the batt. Thus, there is provided a bonded batt, with upper and lower faces, said batt comprising polyester fiberfill of denier per filament about 1 or less, in amount about 75 to about 96% and bonded throughout with lower melting binder material, complementally in amount about 4 to 25%, said amounts being calculated on the basis weight of the batt, said batt having a wash durability (WD, as defined) of at least 4, and a bending stiffness (B, as defined) of about 40 cN/cm<sup>2</sup> or less, wherein at least one of said faces is sealed with a resin having a glass

transition temperature (Tg) of about 0 deg Celsius or less, and preferably from about 0 degrees down to about -30 degrees Celsius, in amount about 0.02 to about 0.35 oz/yd<sup>2</sup>, preferably about 0.1 to about 0.25 oz/yd<sup>2</sup>, calculated with regard to said face of the batt, whereby the sealing rating (SR, as defined) of said face is at least 4. Preferably each of said faces is so sealed.

Both metric units, such as dtex and denier are used herein, 1 dtex being the same as 0.9 denier per filament (dpf).

#### DETAILED DESCRIPTION OF THE INVENTION

Thus, the invention provides fiberfill batts, such as are needed for use in premium apparel, by first preparing a homogeneous blend of polyester fiberfill (70-96% by weight of the blend) and a suitable binder fiber(4-30% by weight of the blend). This blend is converted on a card or garnet to a web which may then be layered or cross lapped to form a batting to whose upper (and preferably serially also to whose lower) face is applied a suitable latex (e.g., a colloidal dispersion of acrylic polymers and/or copolymers in water, discussed in more detail hereinafter), e.g., by spraying. The sprayed batting is heated, e.g., conveniently by being passed through a heated oven to dry the coating(s) and to polymerize the polymeric component(s) to high molecular weight, and to activate the binder fiber. This may be conveniently done, for example, in three passes through such an oven, two to serially dry and partially cure each such coating, after it has been applied to any face, and a final pass to supplement the other(s) and to ensure activation of the binder fiber in preparation for any hot-rolling, in which the bonded batt is passed around or through heated rolls (S-wrap or calendering process) to soften and spread the cured resin and ensure its complete and even distribution among the fibers in the face(s) (large surfaces) of the batt to prevent fiber leakage through such surface(s) of the batt and, if needed, to ensure that the batt is of the desired thickness.

When the fiberfill is of 0.2 to 1 denier per filament, and said resin applied to the batting faces has a glass transition temperature (Tg) of about 0 degrees Celsius and has been applied in amounts between about 0.02 oz/yd<sup>2</sup> (0.7 g/m<sup>2</sup>) to 0.35 oz/yd<sup>2</sup> (12 g/m<sup>2</sup>), then additional treatment, as with hot rolls, is not needed to prevent fiber leakage, especially when dry fiberfill is used. Hot roll treatment may be applied to ensure that the batt is of the desired thickness and to reduce bending stiffness.

The resins that may be used herein are termed variously, by different manufacturers, as "soft" or "medium", or even "very soft", but are characterized by having second order glass transition temperatures (Tg) of about °C. or less, and preferably from about 0 degrees down to about -30 degrees Celsius. They provide both softness and drapability to the batt when used in, e.g., apparel, while acting as barrier to fiber leakage from the batt. The final batts may have a basis weight of 1.5 to 12 oz/yd<sup>2</sup> (50 to 400 g/m<sup>2</sup>) and a thickness of 0.07 to 0.20 inch/oz/yd<sup>2</sup>(0.05 to 0.15 mm/g/m<sup>2</sup>). Thus the batts of this invention are prepared from a blend of polyester fiberfill and binder fibers, and the fibers in the face(s) are sealed by a suitably soft-type resin coating. The polyester fiberfill may all be slickened, e.g., as described herein, or may be a blend of slickened and unslickened fibers. The fiberfill may be solid, hollow, or a blend of solid and hollow fibers and is not limited to any type of fiber cross section, i.e., it may be of cruciform, trilobal, Y-shaped, dog bone, scalloped oval, and other non-circular cross sections as well

as round. The fiberfill has a denier per filament (dpf) within the range of 0.2 to 10, with a dpf of about 1.65 being very useful, and constitutes about 70 to 96% by weight of the blend. As indicated, subdenier fibers give good sealing in the face(s) of the bonded batt, so are often preferred in such face(s). The individual fibers are provided with crimp by conventional means and typically exhibit from 5 to 15 crimps per inch (cpi) and have a length within the range of  $\frac{3}{4}$  to 3 inches. The binder fibers constitute from about 4 to 30% by weight of the batt and may be of the sheath/core (s/c), side/side (s/s), or monocomponent types. These may be obtained from (co)polyesters, polyolefins, polyolefin/polyester, polyamide/polyamide, e.g., and the like. Useful types of binder fibers, and their modes of functioning, are described in, e.g., "Nonwovens World", March/April, 1990, page 37. The initial dpf of suitable binder fibers in the blend is typically within the range of 2 to 15 with a dpf of 4 being commonly used. Useful binder fibers include those disclosed in the aforementioned U.S. Patents to Scott, Pamm, Franckosky, and Marcus, together with those shown in Harris et al U.S. Pat. No. 4,732,809; Taniguchi et al U.S. Pat. No. 4,789,592; Tomioka et al U.S. Pat. No. 4,500,384; Hirose et al Japanese Patent Publication Kokai 57-210,015 (1982); and others known in the art which will function within the oven temperatures disclosed herein. Preferred binder fibers include the commercially-available "Melty 4080" (Unitika Co., Japan) and the "ES" and "EA" polyolefins (Chisso Corporation, Japan).

The cured resin coatings on both faces Of the batt may conveniently constitute about 10 to 30% by weight of the final bonded batt, with 12 to 25% being preferred for 1.65 dpf (1.83 dtex), where lesser amounts of resin tend to reduce wash durability and sealing rating while greater amounts tend to increase stiffness and reduce insulating efficiency. If only one face of the batt is so sealed, only half as much resin need be applied. When low fiber deniers (about 1 dpf or less) are used, less resin coating is needed to achieve fiber leakage control. Moreover, the amount of resin in the surface(s) need not depend on the basis weight of the batting, and so, for heavier battings, the total resin add-on may be as little as 3%, even for slickened fiberfill batts. For entirely dry (unslickened) fibers, less resin is needed than when slickened fiberfill is used.

As noted previously, a suitable sealing resin has a Tg of about 0° C. or less. The useful resins are obtained from commercially-available acrylic and vinyl latex compositions among which are included, e.g., Rhoplex E-32 (Rohm and Haas Co.), TR-934 (Rohm and Haas Co.), X-4280J (Kanebo, Japan), these Hycar® latex compositions of B. F. Goodrich Co.: 26146, 26171, 26322, 26083, 26092, 2671, 26120, 2679, 26796, these latex products of National Starch and Chemical Corporation: NACRYLIC X 4445, NACRYLIC X 788-6007, NACRYLIC X 4483, NACRYLIC X 4460, NACRYLIC X 4260, NACRYLIC X 4425, NACRYLIC X 4465, NACRYLIC 4401, NACRYLIC X 78-3990, NACRYLIC X 78-3997, NACRYLIC X 78-3905, NACRYLIC X 4280, NACRYLIC 4441, NACRYLIC 78-6114, X-LINK 2873, X-LINK 2849, X-LINK 78-6119, X-LINK 2893, X-LINK 2833, X-LINK 78-6004, X-LINK 2813, RESYN 2375, DUR-O-SET E-230, DUR-O-SET E-669, and other commercially-available latexes which are cured to resins whose Tg values are about 0° C. or less. Some of such commercially-available resins and their Tg values are listed in brochures, e.g., one by B. F. Goodrich, dated 1989, entitled HYCAR® Acrylic Latexes, and one by National Starch and Chemical Corporation, entitled Binders, Saturants, Laminants. As the Tg of a

sealing resin gets much lower (than 0° C.), such resins tend to become more sticky. Although such resins can provide good sealing for the surface(s) of the batting, and good wash durability, stickiness of a sealing resin can cause sewing problems, which can require slower sewing speeds, which is not generally preferred. So, the Tg of a sealing resin for use according to the present invention is preferably from about 0° to about -30° C.

Preparation of the batts is generally begun by conventional opening and blending of the polyester fiberfill and binder fiber, followed by carding or garnetting to make a Web. This web can be layered with other webs from a train of cards or garnets, or it can be cross lapped and combined with other webs to form an unbonded batting. This batting is then sprayed with the latex composition on one or both sides of the batting and is fed to the oven for curing of the resin and bonding of the binder fibers. The oven treatment is conducted at 150°-190° C. for 2 to 5 minutes, and may be conveniently done in three passes of the batt, as previously noted. The bonded batt is then passed through/around (preferably at least two) hot rolls having a surface temperature in the range of 150° to 250° C. (more than two rolls may be used). The configuration of the batting may be in S-wrap over the rolls to provide maximum contact with the rolls. The latter may have a clearance of from 2 to 5 mm. depending on the final batting thickness desired. Alternatively, the bonded batting may be passed through calender rolls, heated as above. In these treatments, only one roll may be heated, if desired, even to seal both sides of the batt, which may be passed through/over the rolls a second time to heat the opposite side of the batt, if it is desired to seal both faces. Contact time on the rolls is from 3 to 25 seconds. Such hot roll treatment softens and spreads the resin to ensure its complete and even distribution on the batt surface(s) to prevent fiber leakage and to provide a uniform surface, free of lumps, for comfort and aesthetic performance in use. The batts exhibit the basis weight and thickness ranges previously indicated.

The batts of this invention exhibit desirable levels of thermal resistance or insulation, commonly reported as CLO ratings (see Hwang U.S. Pat. No. 4,514,455). Battts of this invention desirably exhibit a CLO value of at least about 0.36 CLO/oz/yd<sup>2</sup> and preferably 0.48 CLO/oz/yd<sup>2</sup> or higher.

It is to be understood that the components and processes described herein should be selected to provide the batts of this invention. Care must be taken to select combinations that do so provide. For example, the slickener on the fiber and the latex applied to the batt should be selected so as to adhere sufficiently, so that the final batt may exhibit, for example, sufficient wash durability.

#### TEST PROCEDURES

CLO ratings are obtained as described in Hwang, above.

Wash durability ratings ("WD") of the batts of this invention and of comparisons are evaluated by the procedures of ASTM D-4770-88, the panels being 24 inches×24 inches in size, and are reported for measurements made according to paragraph 8.6.1. Battts of the invention exhibit a rating of 3 or higher (paragraph 8.5 scale).

Fiber leakage or percolation through shell fabric is measured as a sealing rating ("SR") by the method described in LeVan U.S. Pat. No. 4,869,771 (after 3 wash cycles unless indicated otherwise), a sealing rating (SR) of 5 being excellent and a sealing rating (SR) of 1 being poor. The batts of this invention exhibit a sealing rating (SR) of 3 or higher

(after 3 wash cycles). In Tables 1 and 3, sealing values are additionally reported after one wash (1 W) as well as after 3 washes (3 W) and compared with initial values before any washing (NEW).

The softness or drapability of the batts of this invention is measured according to German Industrial Standard 53362 Cantilever (DIN 53362 Cantilever) which determines and totals the bending stiffness ("B") of the batting in machine and cross machine directions; the combined results are related to drapability and softness. Batting Test specimens are cut for these measurements to 25 cm. length and 2.5 cm. width, and Test specimens are cut for these measurements in both machine (MD) and cross machine (XD) directions. Each Test specimen is weighed and its weight recorded as "W". Bend length ("LU") is then determined by sliding the Test specimen horizontally on a platform until the front of the bent Test specimen reaches an angle of 41 degrees and 30 seconds. The following calculation is then made:

$$B=F_1(LU/2)^3$$

where B=bending stiffness in cN/cm.<sup>2</sup>

LU=bend length in cm.

$$F_1=9.8 (W/L)$$

W=weight of the specimen sample in grams

L=sample specimen length in cm.

The batts of this invention exhibit a bending stiffness ("B" being the sum of values determined for MD and XD samples from the batt) of 80 cN/cm.<sup>2</sup> or less, a lower bending stiffness being preferred.

The invention is further illustrated in the following Examples, all parts and percentages being by weight, unless otherwise indicated, calculated with regard to the "BW" (Basis Weight, i.e., to the amount of polyester fiberfill and binder fiber only, (i.e., without the added resin sprayed onto the faces to improve the sealing).

#### EXAMPLES

##### Example 1

An 82 lb. sample of polyester staple containing 50 weight percent silicon-slickened fiber of 1.65 dpf (1.83 dtex) and 2 inch cut length and 50 weight percent dry (no slickener) fiber of the same denier and cut length was opened by a conventional mechanical opener and fed to a hopper. In a separate opener was placed 18 lb. of "Melty 4080" binder fiber (4 dpf, 2 inch cut length, 50/50 s/c) which had been pre-opened. The binder fiber was fed to the same hopper containing the staple blend and the fibers were mixed, first by hand, then by mechanical tumbling of the combined actions of the inclined and horizontal aprons.

The mixed fibers were fed to two separate garnets which each produced a continuous web about 60 inches wide and having a basis weight of about 1 oz./yd.<sup>2</sup> (34 g/m.<sup>2</sup>). Each web was passed through a separate cross lapper which produced a cross lapped batt which was placed on a moving conveyor whose speed was about 8 yd./min (7.3 m./min.). The conveyor collected and combined both cross lapped batts into a final multiple-layered batt having a basis weight of about 2.7 oz./yd.<sup>2</sup> (90 g./m.<sup>2</sup>). In a continuous operation, this batt was passed into a spray zone where Kanebo's X-4280J latex (Tg of -4° C.) was applied to the top side of the batt which was then passed into a 3-path oven (sufficient latex was applied to provide 9% by weight cured resin on the batt). This path was at 150° C. and the resin was cured and the binder fiber activated during a residence time of about 1 minute in the oven. After the batt exited the oven, it was

inverted, latex applied to the top side ("new") of the batt, and the batt was carried by a second conveyor to a second path of the oven (170° C.) to cure the resin and activate the binder fiber (resin at 9% by weight resulted on this side of the batt to make a total of 18% by weight resin on the batt). The batting was fed to the third path of the oven (170° C.) to provide further heating of the batt for an additional minute (total heating is for 3 minutes).

The bonded batt is passed through a pair of hot rolls in S-wrap configuration (roll surfaces at 200° C.), with a roll contact time of about 12 seconds; roll separation was 2 mm. The batting is compressed to about one half its original thickness and is wound up into a roll. This batting (18% resin, 18% binder fiber) had a basis weight of 3.33 oz/yd<sup>2</sup>, a thickness of 0.41 inch, exhibited a wash durability (WD) rating of 4, a sealing rating (SR) of 5, and total bending stiffness (B) of 22.1 cN/cm.<sup>2</sup> (MD=8.6, XD=13.5).

#### COMPARATIVE DATA

The following comparisons were carried out to show the unexpected benefit according to the present invention, comparing the effect of using, as sealing resin, one with a Tg of less than about 0° C. (Kanebo's X-4280J, Tg of -4° C.) being compared with the acrylic polymer resin-bonding agent (TR-407, available commercially from Rohm and Haas) used by LeVan in his Example in U.S. Pat. No. 4,869,771 (col. 3, lines 38-39), and having a Tg listed as 34° C.

The fiber used for, the comparative data was a blend of 55% 5.5 denier×2.5 inch slick, 27% 1.65 denier×2.5 inch slick, and 18% 4 denier×2.5 inch "Melty 4080" binder fiber. The process used to make the batting was the same as in Example 1, except that the "Melty 4080" binder fibers had already been combined with the fiberfill, as in Example 2, hereinafter. The blended fibers were opened and were fed to two separate garnets which each produced a continuous web about 60 inch wide and having a basis weight of about 1 oz/yd<sup>2</sup> (34 g/m<sup>2</sup>). Each web was passed through a separate cross-lapper which produced a cross-lapped batt which was placed on a moving conveyor whose speed was about 8 yd/min (7.3 m/min). The conveyor collected and combined both cross-lapped batts into a final multiple-layered batt having a basis weight of 3.7 oz/yd<sup>2</sup> (123 g/m<sup>2</sup>). In a continuous operation, this batt was passed into a spray zone where latex (Kanebo X-4280J for "INV", and R&H TR-407 for "COMP") was applied to the top side of the batt which was then passed into a 3-path oven (sufficient latex was applied to provide 9% by weight cured resin on the batt). This path was at 150° C. and the resin was cured and the binder fiber activated during a residence time of about 1 minute in the oven. After the batt exited the oven, it was inverted, latex applied to the top side (new) of the batt, and the batt was carried by a second conveyor to a second path of the oven (170° C.) to cure the resin and activate the binder fiber (resin at 9% by weight resulted on this side of the batt

to make a total of 18% by weight resin on the batt). The batting was fed to the third path of the oven (170° C.) to provide further heating of the batt for an additional minute (total of heating times was about 3 minutes).

The bonded batt was passed through (for INV and COMP A), or by-passed (for COMP B), a pair of hot rolls in s-wrap configuration (roll surfaces at 200° C.) with a roll contact time of about 12 seconds; roll separation was 3 mm. The batting was compressed to about one half its original thickness and wound up into a roll. These battings had a basis weight of 4.5 oz/yd<sup>2</sup> (150 g/m<sup>2</sup>), a thickness of 0.76 inch (1.93 cm) without "hot roll", and a thickness of 0.59 inch (1.5 cm) with "hot roll". The sealing rates (SR) are listed in Table 1.

TABLE 1

| ITEM NO. | TG<br>(°C.) | ROLL | SEALING RATINGS (SR) |     |     |
|----------|-------------|------|----------------------|-----|-----|
|          |             |      | NEW                  | 1 W | 3 W |
| INV      | -4          | Yes  | 5                    | 5   | 5   |
| COMP A   | +34         | Yes  | 5                    | 5   | 3   |
| COMP B   | +34         | No   | 5                    | 3   | 2   |

Table 1 shows that the Sealing Ratings (SR) for all 3 batts were initially 5, i.e., excellent, and that the SR for the batt of the invention (INV) remained excellent, at 5, even after 3 wash cycles, but that neither of the other batts (COMP A and COMP B, using TR-407, selected by LeVan) had SR values of 5 after 3 wash cycles.

This improvement obtained for batts of invention was not expected.

#### Example 2

In Table 2 are reported the properties of other batts of the invention, prepared by the apparatus and processes described in Example 1, above, using the same latex (Tg of -4° C.), oven and roll temperatures and times as in Example 1. In the Table, "Fiber A" is the fiber blend of Example 1. In all other indicated "Fibers" ("B", etc.), the binder fiber ("Melty 4080") had already been combined with the fiberfill and was not separately added as shown in Example 1. Fiber B is a 78/22 blend of (1) 5 dtex, solid, round cross-section, 50 mm cut length, polyethylene terephthalate staple bearing a polyalkylene oxide slickener and (2) "Melty 4080" (4 dpf); Fiber C is a 78/7/15 blend of (1) solid, round cross-section, silicone-slickened, 3 dpf polyethylene terephthalate staple, (2) 7-hole hollow round cross-section, silicone-slickened, 5.5 dpf polyethylene terephthalate staple, and (3) "Melty 4080" (4 dpf); and Fiber D is a 75/25 blend of (1) 1.65 dpf solid, round cross-section, silicone-slickened, 2 inch cut length polyethylene terephthalate staple and (2) "Melty 4080" (4 dpf).

TABLE 2

| BATTING |       |        |        | BASIS                 |          |    |    | B    |       |      |  |  |
|---------|-------|--------|--------|-----------------------|----------|----|----|------|-------|------|--|--|
| ITEM    | %     | %      | WEIGHT | THICKNESS             | WD       | SR | MD | CD   | TOTAL |      |  |  |
| NO.     | FIBER | BINDER | RESIN  | (OZ/YD <sup>2</sup> ) | (INCHES) |    |    |      |       |      |  |  |
| 1       | A     | 18     | 25     | 3.14                  | 0.41     | 4  | 5  | 33.5 | 35.6  | 69.1 |  |  |
| 2       | A     | 25     | 18     | 2.86                  | 0.35     | 4  | 5  | 20.1 | 31.1  | 51.2 |  |  |
| 3       | B     | 22     | 12     | 2.76                  | 0.35     | 4  | 5  | 23.1 | 38.1  | 61.2 |  |  |

TABLE 2-continued

| BATTING |   |    | BASIS |       | WEIGHT<br>(OZ/YD <sup>2</sup> ) | THICKNESS<br>(INCHES) | B  |      |      |      |       |
|---------|---|----|-------|-------|---------------------------------|-----------------------|----|------|------|------|-------|
| ITEM    | % | %  | NO.   | FIBER | BINDER                          | RESIN                 | WD | SR   | MD   | CD   | TOTAL |
| 4       | C | 15 | 18    | 3.24  | 0.31                            | 5                     | 5  | 14.9 | 18.8 | 33.7 |       |
| 5       | D | 25 | 18    | 3.08  | 0.33                            | 4                     | 5  | 13.2 | 34.6 | 47.8 |       |

## Example 3

Various batting samples were prepared and tested, with results being shown in Table 3. The binder fiber each time was "Melty 4080" (4 dpf), but different fiberfill fibers were used.

Samples A, B, C and D in this Example 3 were prepared from a commercially-available blend of polyester fibers consisting of 37.5% of slickened 1.65 dpf (finished with a silicone slickener), 37.5% of dry 1.65 dpf (without any silicone slickener), and 25% binder fiber. The blend was processed on conventional card and cross-lapper equipment similar to the equipment as described in Example 1. The resulting battings were fed through a triple-pass oven maintained at about 165° C. The battings (except for A) were sprayed with equivalent amounts of a soft resin (glass transition temperature (Tg) equals -10 deg C.) on each side such that the total resin add-on was as stated in Table 3, based on "BW" the basis weight of the fiber in the batting at this stage which was about 4.5 oz/yd<sup>2</sup> (150 g/m<sup>2</sup>). One side of the batting was sprayed with resin before entering the first pass and the other side was sprayed before entering the second pass. Importantly, the entire batting was exposed to adequate time at a temperature sufficiently high to assure complete cure of the resin and set of the binder fiber (1 minute after the batt has reached 165° C. has generally been sufficient). The battings were then calendered in a separate operation which served to seal the surfaces and reduce loft.

From the Sealing Values in Table 3, it can be seen that, under these conditions, even with 8% resin (Sample B), the effect of calendering did not improve the sealing of the 1.65 dpf fibers batt after 1 wash cycle, and even with 15% resin (Sample C), the sealing was improved after 1 wash cycle, but still inadequate after 3 cycles. At 25% resin, under these conditions, the Sealing Rating of the surface of Sample D was satisfactory (after three wash cycles).

The battings were also tested for fiber leakage by encasing in a fabric with a yarn count of 104×84, and a Frazier air permeability rating of 13.2 cu ft/min at pressure drop of 0.5 inches of water.

Samples E and F were the same as Samples A and D, respectively, except these were tested in a fabric with a yarn count of 102×84 and a Frazier rating of 48. Since 0.7 dpf battings were also tested in a more permeable fabric than for Samples A-D, results on Samples E and F (1.65 dpf) are included in Table 3 to bridge the data between Samples A-D and G-Q. Sample E, without resin, failed when new because of the openness of the fabric, but after three wash cycles had become sufficiently matted that it improved its leakage performance. Sample F's Sealing Value was 5 initially and provided a satisfactory Sealing Rating, i.e., after 3 wash cycles).

Samples G, H, I and J were prepared from a blend of about 85 pounds of dry polyester fibers (0.7 dpf, 0.78 dtex, 1.5 inch cut, 12 cpi, without any special slickening finish) and 15 pounds of binder fiber. These samples were resin-sprayed, calendered and tested as for samples E and F.

Samples K and L were prepared from a blend of about 55 pounds of similar 0.7 dpf slick fiber, finished with a silicone slickener, 27 pounds of dry (unslickened) 0.7 dpf fiber, and 18 pounds of binder fiber. These samples were not calendered, as indicated by the double asterisks in Table 3, but gave good sealing ratings.

Samples M, O, P and Q were similarly prepared from the same kind of blend as K and L, but were made to higher basis weights, as shown, and also showed good sealing ratings, despite lower (less than 10%) resin add-on and despite not being calendered, because of use of low dpf fiber. N was calendered (unlike the others). A comparison of these results shows that calendering was not needed to improve the sealing rating. (when the subdenier fibers were used with the soft resin).

Samples G through L were all tested for fiber leakage using the 48 Frazier fabric.

Accordingly, in Table 3, samples D, F thru I and K thru Q are all according to the invention, whereas A, E and J show comparisons (without any resin sprayed on) and B and C also show comparisons (with regular denier fiberfill) whose sealing ratings are not adequate after washing.

TABLE 3

|     | FRAZIER | BW  | DPF  | FI-BER RESIN |       | SEALING RATINGS |     |     |
|-----|---------|-----|------|--------------|-------|-----------------|-----|-----|
|     |         |     |      | %            | *     | NEW             | 1 W | 3 W |
| A   | 13.2    | 4.5 | 1.65 | 0            | 0     | 5               | 1   | 1   |
| B   | 13.2    | 4.5 | 1.65 | 8            | 0.36  | 5               | 1   | 1   |
| C   | 13.2    | 4.5 | 1.65 | 15           | 0.67  | 5               | 3   | 1   |
| D   | 13.2    | 4.5 | 1.65 | 25           | 1.125 | 5               | 5   | 5   |
| E   | 48      | 4.5 | 1.65 | 0            | 0     | 1               | 1   | 4   |
| F   | 48      | 4.5 | 1.65 | 25           | 1.125 | 5               | 5   | 5   |
| G   | 48      | 4.5 | 0.7  | 4            | 0.18  | 5               | 5   | 5   |
| H   | 48      | 4.5 | 0.7  | 2.2          | 0.10  | 5               | 5   | 5   |
| I   | 48      | 4.5 | 0.7  | 1.6          | 0.07  | 5               | 5   | 5   |
| J   | 48      | 4.5 | 0.7  | 0            | 0     | 4               | 1   | 1   |
| K** | 48      | 4.5 | 0.7  | 10           | 0.45  | 5               | 5   | 5   |
| L** | 48      | 4.5 | 0.7  | 5            | 0.225 | 5               | 5   | 5   |
| M** | 48      | 6.1 | 0.7  | 6            | 0.37  | 5               | 5   | 4   |
| N   | 48      | 5.1 | 0.7  | 7            | 0.36  | 5               | 5   | 5   |
| O** | 48      | 8.0 | 0.7  | 6            | 0.48  | 5               | 5   | 5   |
| P** | 48      | 8.1 | 0.7  | 8            | 0.65  | 5               | 5   | 5   |
| Q** | 48      | 9.3 | 0.7  | 5            | 0.47  | 5               | 5   | 5   |

\*indicates the total amount of resin sprayed on (both surfaces of) the batt, calculated in oz/yd<sup>2</sup> (half these amounts indicate the amounts on each face).

\*\*indicates there was no calendering after oven cure

## Example 4

In the following Table 4 are reported the properties of other batts of the invention, prepared by the apparatus and process essentially as described in Example 2, above, using the same oven and roll temperatures and times as in Examples 1 and 2, but a different latex. The latex used for this Example 4 was Rohm and Haas' Rhoplex ST-954, having a glass transition (Tg) temperature of -23° C. "Fiber

## 11

A" was the same fiber blend as that used in Example 1; the binder fiber ("Melty 4080") had already been combined with the fiberfill. The batts in this Example provided good WD, SR and low bending stiffness (i.e., were desirably soft) as described according to the invention; they tended to become slightly sticky (which can tend to make them more difficult to cut and sew during garment manufacturing, because of the lower Tg, -23° C. of the latex) We believe that a latex with an even lower Tg (less than -30° C.) would generally tend to cause even more stickiness, and so would be even less desirable for normal operation.

## 12

defined) of at least 3, and a bending stiffness (B, as defined) of about 80 cN/cm<sup>2</sup> or less, wherein at least one of said faces is sealed with a resin having a glass transition temperature (Tg) in the range of about 0 degrees to -30 degrees Celsius, 5 in an amount of about 5 to 15% of the total weight of the batt, whereby the sealing rating (SR, as defined) after 3 wash cycles of said face is at least 4.

4. A batt according to claim 3, wherein the bending stiffness is about 50 cN/cm<sup>2</sup> or less.

5. A bonded bait with upper and lower faces, said bait comprising polyester fiberfill of dealer per filament about 1

TABLE 4

| BATTING |       |        |        | BASIS                 |          |    |    |      |      |       |
|---------|-------|--------|--------|-----------------------|----------|----|----|------|------|-------|
| ITEM    | %     | %      | WEIGHT | THICKNESS             | B        |    |    |      |      |       |
| NO.     | FIBER | BINDER | RESIN  | (OZ/YD <sup>2</sup> ) | (INCHES) | WD | SR | MD   | CD   | TOTAL |
| 6       | A     | 18     | 18     | 2.41                  | 0.41     | 4  | 5  | 24.6 | 29.5 | 54.1  |
| 7       | A     | 18     | 18     | 4.37                  | 0.49     | 4  | 5  | 15.3 | 18.9 | 34.2  |

What we claim is:

1. A bonded batt with upper and lower faces, said batt comprising polyester fiberfill of 0.2 to 10 dtex per filament, in an amount of about 75 to 98%, and bonded throughout with lower melting binder material, in an amount of about 2 to 25%, said amounts being calculated on the basis weight of the batt, said upper and lower faces of said batt being sealed with a resin having a glass transition temperature (Tg) in the range of about 0 degrees to -30 degrees Celsius, in an amount of about 10 to 30% of the total weight of the batt, whereby the sealing rating (SR, as defined) after 3 wash cycles of said faces is at least 4, said batt having a wash durability (WD, as defined) of at least 3, and a bending stiffness (B, as defined) of about 80 cN/cm<sup>2</sup> or less.

2. A batt according to claim 1, wherein the bending stiffness is about 50 cN/cm<sup>2</sup> or less.

3. A bonded batt with upper and lower faces, said batt comprising polyester fiberfill of 0.2 to 10 dtex per filament, in an amount of about 75 to 98%, and bonded throughout with lower melting binder material, in an amount of about 2 to 25%, said amounts being calculated on the basis weight of the batt, said batt having a wash durability (WD, as

25 defined) of at least 4, and a bending stiffness (B, as defined) of about 40 cN/cm<sup>2</sup> or less, wherein at least one of said faces is sealed with a resin having a glass transition temperature (Tg) in the range of about 0 degrees to -30 degrees Celsius, in amount about 0.02 oz/yd<sup>2</sup> to about 0.35 oz/yd<sup>2</sup>, calculated with regard to said face of the batt, whereby the sealing rating (SR, as defined) after 3 wash cycles of said face is at least 4.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530

UNITED STATES PATENT AND TRADEMARK OFFICE  
**CERTIFICATE OF CORRECTION**

PATENT NO. : 5,527,600  
DATED : June 18, 1996  
INVENTOR(S) : Michael S. Frankosky; Wo K. Kwok

It is certified that error appears in the above-identified patent and that said Letters Patent is hereby corrected as shown below:

Col. 12, line 3,

In Claim 3, line 9, "rosin" is hereby deleted and -- resin -- is inserted in place thereof.

Col. 12, line 10,

In Claim 5, line 1, "bait" is hereby deleted and -- batt -- is inserted in place thereof.

Col. 12, line 11,

In Claim 5, line 2, "dealer" is hereby deleted and -- denier -- is inserted in place thereof.

**Signed and Sealed this**

**Seventh Day of January, 1997**

*Attest:*



BRUCE LEHMAN

*Attesting Officer*

*Commissioner of Patents and Trademarks*